



US00560988A

## United States Patent [19]

Uda et al.

[11] Patent Number: 5,609,888

[45] Date of Patent: Mar. 11, 1997

## [54] APPARATUS FOR PRODUCING MULTIFILAMENTS

[75] Inventors: **Hitoshi Uda; Tetsuya Takahashi; Ryosuke Kamei; Takeshi Sano**, all of Kanagawa, Japan[73] Assignee: **Showa Denko Kabushiki Kaisha**, Tojyo, Japan

[21] Appl. No.: 444,029

[22] Filed: May 18, 1995

## Related U.S. Application Data

[60] Continuation of Ser. No. 132,254, Oct. 6, 1993, abandoned, which is a division of Ser. No. 0,099, Jan. 4, 1993, Pat. No. 5,283,025.

## [30] Foreign Application Priority Data

Jan. 9, 1992 [JP] Japan ..... 4-2216  
Feb. 4, 1992 [JP] Japan ..... 4-19108[51] Int. Cl.<sup>6</sup> ..... D01D 5/088; D01D 5/092; D01D 5/16

[52] U.S. Cl. ..... 425/66; 264/210.8; 264/211.15; 264/211.17; 264/237; 425/72.2

[58] Field of Search ..... 264/24, 168, 237, 264/210.8, 211.14, 211.15, 211.17, 210.7; 425/72.1, 72.2, 76, 7, 66

## [56] References Cited

## U.S. PATENT DOCUMENTS

3,054,652 9/1962 Heumann ..... 264/28  
3,271,943 9/1966 Williams ..... 264/168  
3,489,832 1/1970 Bruton et al. ..... 264/237  
3,511,905 5/1970 Martin ..... 264/210.8

|           |         |                       |            |
|-----------|---------|-----------------------|------------|
| 3,672,013 | 6/1972  | Vernon et al. ....    | 425/66     |
| 3,790,995 | 2/1974  | Martin et al. ....    | 425/66     |
| 3,832,435 | 8/1974  | Bauer et al. ....     | 264/168    |
| 3,995,004 | 11/1976 | Heinrich et al. ....  | 264/237 X  |
| 4,200,602 | 4/1980  | Grayson ....          | 24/210.8   |
| 4,244,907 | 1/1981  | Wu ....               | 264/168    |
| 4,301,102 | 11/1981 | Fernstrom et al. .... | 264/168    |
| 4,461,740 | 6/1984  | Koschinek et al. .... | 425/66     |
| 4,522,774 | 6/1985  | Donnelly et al. ....  | 264/168    |
| 4,863,662 | 9/1989  | Hasegawa et al. ....  | 264/130    |
| 4,902,462 | 2/1990  | Bert ....             | 264/211.13 |
| 5,238,025 | 2/1994  | Uda et al. ....       | 264/211.17 |

## FOREIGN PATENT DOCUMENTS

|           |         |                         |
|-----------|---------|-------------------------|
| 0285736   | 10/1988 | European Pat. Off. .... |
| 2155207   | 5/1972  | Germany .               |
| 3539185   | 5/1986  | Germany .               |
| 3540181   | 7/1986  | Germany .               |
| 56-4731   | 1/1981  | Japan .                 |
| 61-152840 | 7/1986  | Japan .                 |
| 2101522   | 1/1983  | United Kingdom .        |

Primary Examiner—Jay H. Woo

Assistant Examiner—Duane S. Smith

Attorney, Agent, or Firm—Sughrue, Mion, Zinn, Macpeak &amp; Seas

## [57] ABSTRACT

An apparatus for producing multifilaments having high fiber strength is disclosed. A spinneret melt spins a polyolefin at a first temperature into filaments. A cooling duct cools the filaments via convection at a second temperature. A chill roll, disposed downstream from the cooling duct, has a third temperature, and forcibly conductively cools the filaments. Finally, heated drawing rolls, disposed downstream from said chill roll, continuously draw the filaments at a high draw ratio.

21 Claims, 1 Drawing Sheet



FIG. 1



FIG. 2



## APPARATUS FOR PRODUCING MULTIFILAMENTS

This is a Continuation of application Ser. No. 08/132,254 filed Oct. 6, 1993, now abandoned, which is a divisional of application Ser. No. 08/000,099, filed Jan. 4, 1993, now U.S. Pat. No. 5,283,025.

### BACKGROUND OF THE INVENTION

The present invention relates to a method for producing multifilaments. Multifilaments formed of polyolefins such as polypropylene and polyethylene are used to make pile yarns for ropes, nets, and carpets or as raw yarns for nonwoven fabrics.

In general, to manufacture multifilaments from thermoplastic resins, a number of molten filaments extruded through a spinneret are cooled in an ambient air stream by passage through a cooling duct less than 3-5 m long as they are taken up with drafting being effected at a comparatively high speed of approximately 300 m/min. Thereafter, the filaments are drawn, crimped, and otherwise processed in separate steps.

With the recent improvement in the performance of winders, a method called "direct spin and draw" has been proposed to perform a continuous process including the steps of spinning, drawing, and crimping. However, this method is incapable of producing high-strength multifilaments having satisfactory fiber strength.

### SUMMARY OF THE INVENTION

An object, therefore, of the present invention is to provide a process for producing high-strength polyolefinic multifilaments by the direct spin and draw method.

In order to develop a process for producing high-strength polyolefinic multifilaments by the direct spin and draw method, the present inventors conducted intensive studies and found that their objective could be attained by a process comprising the steps of melt spinning a polyolefin, cooling the spun filaments with air by passage through a cooling duct, cooling the filaments with a chill roll having a surface temperature of 5°-30° C. and then continuously drawing the filaments at high draw ratio in-line with a heating roll having a surface temperature of 80°-150° C.

Examples of the polyolefin that can be used in the present invention include low-density polyethylene, medium-density polyethylene, high-density polyethylene, polypropylene, poly-1-butene and poly-4-methylpentene-1. Any polyolefins may be used as long as they can be molded into filament assemblies by melt extrusion and there is no particular limitation on such factors as the molecular weight, density and molecular weight distribution. Nevertheless, in case of polypropylenes, it is preferable to use the polypropylenes having a narrow molecular distribution which meet the following condition:

$$M_w/M_n < 7.0$$

where  $M_w$  is the weight-average molecular weight and

$M_n$  is the number-average molecular weight.

According to the invention, there is provided a process for producing multifilaments, comprising the steps of: melt spinning a polyolefin at a first temperature; cooling the spun filaments with a first chill means which is of a non-contact type and is held at a second temperature; cooling the filaments at a third temperature with a second chill means

which is of a contact type for forcibly cooling the filaments; and drawing continuously the filaments at high draw ratio in-line with heating rolls having a predetermined surface temperature so that the filaments cooled at said third temperature are directly and continuously treated by said heating rolls.

According to another aspect of the invention, there is provided an apparatus for producing multifilaments, comprising: means for melt spinning a polyolefin at a first temperature; first chill means for cooling the spun filaments, said first chill means being of a non-contact type and is held at a second temperature; second chill means for cooling the filaments at a third temperature, said second chill means being of a contact type for forcibly cooling the filaments; and means for drawing continuously the filaments at high draw ratio in-line with heating rolls having a predetermined surface temperature, said drawing means being located in series with said second chill means.

### BRIEF DESCRIPTION OF THE DRAWINGS

In the accompanying drawings:

FIG. 1 is a schematic view showing an apparatus for implementing a method according to the present invention; and

FIG. 2 is a schematic view showing another apparatus for implementing another method according to the present invention.

### DESCRIPTION OF THE PREFERRED EMBODIMENTS

A first method of the present invention is described below.

FIG. 1 shows an example of the apparatus that can be used to implement the present invention. A polyolefin is extruded from an extruder (not shown) through a spinning nozzle 1 to produce undrawn multi-filaments 3. The shaping temperature is desirably as high as possible on the condition that filament assemblies can be produced without causing deterioration of the polyolefin. The spinning nozzle 1 is preferably such that the extruded filaments can be cooled uniformly.

The spun but undrawn multifilaments are cooled to solidify by passage through a cooling duct 2. Cooling may be performed to such an extent that the individual filaments will not fuse together, with the temperature in the cooling duct being desirably adjusted to lie within the range of 5°-40° C. and with air being supplied at a flow rate of 0.1-0.5 m/sec. After cooling, the filaments are treated with oil or gathering agent by means of an oiling roller 4.

The oil treated multifilaments are then cooled with chill rolls 5. The chill rolls 5 are typically godets but other rolls such as nip rolls may be used. The chill rolls 5 may be of Nelson roll type including a pair of rolls which are arranged with their rotary axes being somewhat offset from each other in order to prevent the filaments from being locally wound around the rolls. The chill rolls 5 must have a surface temperature of 5°-30° C., preferably, 5°-20° C. which is maintained by cooling control device 10.

The surface temperature of the chill rolls 5 has a substantial effect on the linear strength of the multifilaments. The use of takeup rolls has been known but they have not been used to achieve positive cooling as in the present invention and it has been entirely unknown that positive conductive cooling is effective in achieving marked improvements in the physical properties of multifilaments.

Suitable cooling media are water, brine, etc., and they are desirably supplied in a circulating system.

The multifilaments cooled with the chill rolls **5** are drawn on heating rolls **6-1** and **6-2** and the drawn multifilaments **8** are cooled on a chill godet roll **7** and thereafter wound up as the product on take up roll **9**. The heating roll may be a godet roll, nip rolls, etc. In this case, it is preferable to make surfaces of the heating rolls **6-1** and **6-2** mirror-finished in order to increase contact area between the filaments and roll surfaces. Drawing may be performed in multiple stages. The drawing temperature is typically in the range of 80°–150° C., with range of 100°–140° C. being particularly preferred. Drawing is preferably effected at a high draw ratio of 8–15. If the draw ratio is less than 8, only multifilaments of low strength are produced. On the other hand, it is difficult to perform drawing at draw ratios exceeding 15.

### EXAMPLES

#### Example 1

In the apparatus shown in FIG. 1, a polypropylene having MFR of 7.8/10 min (ASTM D 1238, L) (molecular distribution Mw/Mn of 4.0) available from Showa Denko K. K. under the trade name "SHOWALLOMER TA 553-4" was extruded from an extruder (40 mm in diameter) through a multifilament spinning nozzle having 68 holes (0.6 in diameter) at an extrusion temperature of 280° C. in a throughput of 35 g/min. The undrawn multifilaments as the extrudates were passed through a cooling duct 900 mm long, in which they were cooled with air at a temperature of 18° C. that was flowing at a velocity of 0.5 m/sec. The cooled filaments were treated with an oil by means of an oiling roller and thereafter cooled with a godet roll that was held at a surface temperature of 15° C. by means of circulating water and which was rotating at a peripheral speed of 35 m/min. Subsequently, the filaments were heated on a pair of draw rollers having a surface temperature of 120° C. and wound up at a speed of 300 m/min. The multifilaments thus produced were found to have a linear strength of 8.0 g/d and an elongation of 14%.

#### Example 2

The procedure of Example 1 was repeated except that the chill godet roll was held at a surface temperature of 5° C. The multifilaments produced were found to have linear strength of 9.0 g/d and an elongation of 12%.

#### Example 3

A polypropylene having MFR of 14 g/10 min (ASTM D 1238, L) (molecular distribution Mw/Mn of 6.2) available from Showa Denko K. K. under the trade name "SHOWALLOMER MH510H" was extruded from an extruder (40 mm in diameter) through a multifilament spinning nozzle having 68 holes (0.6 in diameter) at an extrusion temperature of 280° C. in a throughput of 35 g/min. The undrawn multifilaments as the extrudates were passed through a cooling duct 900 mm long, in which they were cooled with air at a temperature of 18° C. that was flowing at a velocity of 0.5 m/sec. The cooled filaments were treated with an oil by means of an oiling roller and thereafter cooled with a godet roll that was held at a surface temperature of 15° C. by means of circulating water and which was rotating at a peripheral speed of 35 m/min. Subsequently, the filaments were heated on a pair of draw rollers having a surface temperature of 120° C. and wound up at a speed of 210

m/min. The multifilaments thus produced were found to have a linear strength of 5.9 g/d and an elongation of 33%.

#### Example 4

A polypropylene having MFR of 2.5 g/10 min (ASTM D 1238, L) (molecular distribution Mw/Mn of 5.1) available from Showa Denko K. K. under the trade name "SHOWALLOMER TA253" was extruded from an extruder (40 mm in diameter) through a multifilament spinning nozzle having 68 holes (0.6 in diameter) at an extrusion temperature of 280° C. in a throughput of 35 g/min. The undrawn multifilaments as the extrudates were passed through a cooling duct 900mm long, in which they were cooled with air at a temperature of 18° C. that was flowing at a velocity of 0.5 m/sec. The cooled filaments were treated with an oil by means of an oiling roller and thereafter cooled with a godet roll that was held at a surface temperature of 15° C. by means of circulating water and which was rotating at a peripheral speed of 50 m/min. Subsequently, the filaments were heated on a pair of draw rollers having a surface temperature of 120° C. and wound up at a speed of 370 m/min. The multifilaments thus produced were found to have a linear strength of 7.6 g/d and an elongation of 27%.

#### Example 5

A polypropylene having MFR of 330 g/10 min (ASTM D 1238, L) (molecular distribution Mw/Mn of 4.9) available from HH441 (made by HIMONT company) was extruded from an extruder (40 mm in diameter) through a multifilament spinning nozzle having 68 holes (0.6 in diameter) at an extrusion temperature of 200° C. in a throughput of 20 g/min. The undrawn multifilaments as the extrudates were passed through a cooling duct 900 mm long, in which they were cooled with air at a temperature of 18° C. that was flowing at a velocity of 0.2 m/sec. The cooled filaments were treated with an oil by means of an oiling roller and thereafter cooled with a godet roll that was held at a surface temperature of 15° C. by means of circulating water and which was rotating at a peripheral speed of 50 m/min. Subsequently, the filaments were heated on a pair of draw rollers having a surface temperature of 110° C. and wound up at a speed of 300 m/min. The multifilaments thus produced were found to have a linear strength of 4.6 g/d and an elongation of 15%.

#### Comparative Example 1

The same resin as used in Example 1 was spun into filaments. After treatment with an oil, the filaments were not passed around the chill godet roll **5** at a speed of 35 m/min but they were directly passed between the pair of draw rollers to be drawn at a temperature of 120° C. A maximum draw speed that could be achieved was only 140 m/min. The multifilaments thus produced were found to have a linear strength of only 3.8 g/d and an elongation of 140%.

#### Comparative Example 2

The procedure of Example 1 was repeated except that the chill godet roll was held at a surface temperature of 40° C. The multifilaments produced were found to have a strength of only 3.5 g/d and an elongation of 170%.

#### Comparative Example 3

The same resin as used in Example 5 was spun into filaments. After treatment with an oil, the filaments were not passed around the chill godet roll **5** at a speed of 50 m/min

but they were directly passed between the pair of draw rollers to be drawn at a temperature of 110° C. A maximum draw speed that could be achieved was only 140 m/min. The multifilaments thus produced were found to have a linear strength of only 2.2 g/d and an elongation of 80%.

The process of the present invention allows high-strength multifilaments to be produced by the direct spin and draw method without performing spinning and drawing in two separate steps.

Multifilaments of high strength and low elongation can be produced without performing spinning and draw in two separate steps.

FIG. 2 shows another example of the apparatus that can be used to implement the present invention. In the same way as the previous embodiment, a polyolefin is extruded from an extruder through a spinning nozzle 1 to produce undrawn multi-filaments 3.

The shaping temperature is desirably as high as possible on the condition that filament assemblies can be produced without causing deterioration of the polyolefin; that is, the polyolefin to be used is spinnable but non-decomposed.

The spinning nozzle 1 is preferably such that the extruded filaments can be cooled uniformly.

The spun but undrawn multifilaments are cooled to solidify by passage through a cooling duct 2. Cooling may be performed to such an extent that the individual filaments will not fuse together, with the temperature in the cooling duct being desirably adjusted to lie within the range of 5°-40° C. and with air being supplied at a flow rate of 0.1-0.5 m/sec.

The undrawn multifilaments cooled by passage through the cooling duct 2 are then quenched and supplied with a gathering agent by means of a gathering agent supply roller 4. This roller must have a temperature of 0°-10° C., with the range of 0-5° C. being preferred, which is maintained by cooling control device 11. The gathering agent to be used is not limited in any particular way as long as it will neither solidify nor deteriorate at temperature of 0°-10° C.

The temperature of the gathering agent supply roller 4 has a substantial effect on the linear strength of the multifilaments.

The use of roller 4 for supplying a gathering agent has been known but they have not been used to achieve positive conductive cooling as in the present invention and it has been entirely unknown that positive conductive cooling is effective in achieving marked improvements in the physical properties of multifilaments.

Suitable cooling media are water, brine, etc, and they are desirably supplied in a circulating system.

The multifilaments 8 cooled with the roll 4 are drawn on heating rolls 6-1 and 6-2 and the drawn multifilaments are cooled on a chill godet roll 7 and thereafter wound up as the product on a takeup roll 9. The heating rolls 6-1 and 6-2 may be godet rolls, nip rolls, etc. Drawing may be performed in multiple stages. The drawing condition may be substantially the same as the previous method implemented by the apparatus shown in FIG. 1.

#### Example 6

In the apparatus shown in FIG. 2, a polypropylene having MFR of 7.8/10 min (ASTM D 1238, L) (molecular distribution Mw/Mn of 4.0) available from Showa Denko K. K. under the trade name "SHOWALLOMER TA 553-4" was extruded from an extruder (40 mm in diameter) through a

multifilament spinning nozzle having 68 holes (0.6 in diameter) at an extrusion temperature of 280° C. in a throughput of 120 g/min.

The undrawn multifilaments as the extrudates were passed through a cooling duct 900 mm long, in which they were cooled with air at a temperature of 18° C. that was flowing at a velocity of 0.5 m/sec. The filaments were quenched and supplied by the cooling gathering agent supply roller which was rotated at a peripheral speed of 3 m/min and which was cooled at 5° C. with gathering agents. Subsequently, the filaments were heated on a pair of draw rollers having a surface temperature of 120° C. and wound up at a speed of 300 m/min so that the filaments were drawn at a speed of 2,000 m/min. The multifilaments thus produced were found to have a linear strength of 7.0 g/d and an elongation of 20%.

#### Example 7

The procedure of Example 6 was repeated except that the gathering agent supply roller roll was cooled at 10° C. and that the filaments were drawn at a speed of 1,500 m/min. The multifilaments produced were found to have linear strength of 6.0 g/d and an elongation of 40%.

#### Comparative Example 4

The same resin as used in Example 6 was spun into filaments which were supplied with a gathering agent from a roller that was not cooled. In the subsequent drawing step, the draw speed could be raised to only 1,000 m/min. The multifilaments thus produced were found to have a linear strength of only 3.5 g/d and an elongation of 150%.

The process of the present invention allows high-strength multifilaments to be produced by the direct spin and draw method without performing spinning and drawing in two separate steps.

What is claimed is:

1. An apparatus for producing multifilaments having high fiber strength, comprising:
  - a melt-spinning device which melt spins a polyolefin at a first temperature into filaments;
  - a first chill device, disposed downstream from said melt-spinning device, which cools the spun filaments, said first chill device being a non-contact device and having a second temperature;
  - a gathering device, disposed downstream of said first chill device, which gathers said filaments to provide a gathered fiber;
  - a second chill device, disposed downstream from said first chill device and said gathering device, having a third temperature within a range of 5° to 30° C., said second chill device forcibly conductively cooling the gathering fiber;
  - a cooling control device which maintains said second chill device at said third temperature; and
  - heated drawing rolls, disposed downstream from said second chill device, which continuously draw the gathered fiber at a high draw ratio to produce said multifilaments, said heated drawing rolls having a predetermined surface temperature;
  - said melt-spinning device, first chill device, gathering device, second chill device, cooling control device and heated drawing rolls cooperating so that said multifilaments have said high fiber strength which is in a range of 4.6 to 8.0 g/d.

2. The apparatus according to claim 1, wherein said first chill device comprises a cooling duct through which the filaments pass.

3. An apparatus for producing multifilaments having high fiber strength, comprising:

a melt-spinning device which melt spins a polyolefin at a first temperature into filaments;

a first chill device, disposed downstream from said melt-spinning device, which cools the spun filaments, said first chill device being a non-contact device and having a second temperature;

a gathering and chill device, disposed downstream from said first chill device, having a third temperature within a range of 0° to 10° C., said gathering and chill device gathering said filaments to provide a gathered fiber and forcibly conductively cooling the gathered fiber;

a cooling control device which maintains said gathering and chill device at said third temperature; and

heated drawing rolls, disposed downstream from said gathering and chill device, which continuously draw the gathered fiber at a high draw ratio to produce said multifilaments, said heated drawing rolls having a predetermined surface temperature;

said melt-spinning device, first chill device, gathering and chill device, cooling control device and heated drawing rolls cooperating to produce said multifilaments having said high fiber strength which is in a range of 4.6 to 8.0 g/d.

4. The apparatus according to claim 2, wherein said first temperature is in the range of 190° to 290° C.

5. The apparatus according to claim 3, wherein said first temperature is in the range of 190° to 290° C.

6. The apparatus according to claim 1, wherein the predetermined surface temperature of said heated drawing rolls is in the range of 80° to 150° C.

7. The apparatus according to claim 1, wherein said high draw ratio is in the range of 8-15.

8. The apparatus according to claim 1, wherein said gathering device is a gathering roller.

9. The apparatus according to claim 1, wherein second chill device is a chill roller.

10. The apparatus according to claim 1, wherein the gathering device applies a gathering agent to the filaments.

11. The apparatus according to claim 1, wherein the third temperature is within a range of 5° to 15° C.

12. The apparatus according to claim 3, wherein the gathering and chill device is a chill and gathering roller.

13. The apparatus according to claim 3, wherein the gathering and chill device applies a gathering agent to the filaments.

14. The apparatus according to claim 3, wherein the third temperature is in a range of 0° to 5° C.

15. The apparatus according to claim 3, wherein said first chill device comprises cooling duct through which the filaments pass.

16. The apparatus according to claim 3, wherein the predetermined surface temperature of said heating rolls is in the range of 80° to 150° C.

17. The apparatus according to claim 3, wherein said high draw ratio is in the range of 8-15.

18. The apparatus according to claim 1, further comprising a third chill device, disposed downstream from said heated drawing rolls, for forcibly conductively cooling the multifilaments.

19. The apparatus according to claim 18, wherein the third chill device is a chill roller.

20. The apparatus according to claim 3, further comprising a second chill device, disposed downstream from said heated drawing rolls, for forcibly conductively cooling the multifilaments.

21. The apparatus according to claim 20, wherein the second chill device is a chill roller.

\* \* \* \* \*